

June 14, 1927.

C. A. BRAUCHLER

1,632,533

PROCESS OF FORGING GEAR BLANKS

Filed Oct. 4, 1922

3 Sheets-Sheet 1



Fig. 1



Fig. 3



Fig. 2

Inventor

By C. A. Brauchler

Grease and Bond Attorney

June 14, 1927.

1,632,533

C. A. BRAUCHLER

PROCESS OF FORGING GEAR BLANKS

Filed Oct. 4, 1922

3 Sheets-Sheet 2



Fig. 6

Fig. 4

Inventor

C. A. Brauchler

334 *Grease my Bond*

Attorneys

June 14, 1927.

1,632,533

C. A. BRAUCHLER

PROCESS OF FORGING GEAR BLANKS

Filed Oct. 4, 1922

3 Sheets-Sheet 3

Fig. 7



Fig. 8



Inventor

C. A. Brauchler

By Grease and Bond

Attorneys

## UNITED STATES PATENT OFFICE.

CHARLES A. BRAUCHLER, OF CANTON, OHIO.

## PROCESS OF FORGING GEAR BLANKS.

Application filed October 4, 1922. Serial No. 592,276.

This invention relates to forged metal gear blanks and a process of forging the same and has for its objects to produce a gear blank from a blank cut from a metal bar, in which the teeth of the finished gear will be made from metal originally at the surface of the bar, the grain of the metal flowing from the center to the periphery of the wheel and back toward the center.

It is well known that the center of any bar of steel is the least refined portion of the same, due to the fact that being the most remote from the surface, it receives the least working during the working of the bar. For this reason, the greatest amount of defects and impurities are always located through the axial center of a steel bar.

It is also well known that all bar steel has a grain running parallel to the direction of rolling or axis of the bar, this grain being closer and more refined around the periphery of the bar, while in the central portion of the bar, the grain is comparatively coarse.

The invention may be attained by cutting or "cracking" a blank from a steel bar, the blank being of a length greater than its diameter, heating the blank, and upsetting the same endwise to produce a barrel shaped or double truncated cone and then placing the partly completed product in a forging die and forging the gear blank therein, the outside grain of the metal thus being caused to flow outward around the periphery of the gear blank, placing the most refined portion of the grain in the portion of the gear blank from which the teeth are cut, this, of course, being the portion of the gear which stands the greatest wear, while the center of the gear which requires the least strength and is often removed altogether, is formed from the central portion of the bar which has the least refinement and which contains the greatest amount of defects and impurities.

A preferred embodiment of the invention is illustrated in the accompanying drawings, in which—

Figure 1 is a perspective view of the blank from which the gear blank is formed;

Fig. 2, a sectional view through the upsetting and forging dies by means of which the gear blank is formed;

Fig. 3, a detail sectional view of the up-

setting die, showing the same in the open position, a blank being located therein;

Fig. 4, a similar view showing the upsetting die in the closed position, the partly completed product being shown in section; 60

Fig. 5, a detail sectional view of the forging die showing the same in the open position, the upset blank being shown in position therein;

Fig. 6, a view of the forging die in the 65 closed position, the finished gear blank being shown in section therein;

Fig. 7, an enlarged, transverse, sectional view of the finished gear blank; and

Fig. 8, a similar view of the finished gear 70 formed therefrom.

Similar numerals indicate corresponding parts throughout the drawings.

In Fig. 1 a blank is illustrated at 1 which is cut, "cracked" or otherwise severed from 75 a rolled bar in a manner to produce square or flat ends upon the blank as at 2. It will be noted that the blank is of a length considerably greater than its diameter, this being preferable in order that the grain of 80 the metal may flow properly when the blank is forged in the dies, as hereinafter described.

The dies in which the gear blank is formed are preferably of the form shown in 85 Fig. 2, and comprise the upper and lower die blocks 3 and 4 respectively, the lower block being fixed and the upper block arranged to reciprocate by means of a hammer or the like. These blocks are provided with 90 the upsetting die 5 and the forging die 6 located adjacent to each other to facilitate the forming of the gear blank, the uncompleted product being removed from the upsetting die and placed in the forging die 95 while still hot for the finishing operation.

The upsetting die comprises the lower inverted frusto-conical portion 7 and the upper frusto-conical portion 8 registering therewith and provided at its top with a centering point 9. As shown in Fig. 3, the grain of the blank 1 is refined around the periphery as indicated at 10, while the grain through the central portion of the blank as shown at 11 is less refined and contains 105 impurities and imperfections.

It is the intention of the present invention to cause the more refined grain at the periphery of the blank to flow outward from the center, placing the same in the portion 110

of the gear blank from which the teeth are cut, while the less refined grain remains at the axial center of the gear blank, at the point where the least strain and wear is placed upon the gear.

As shown in Fig. 3, the reduced bottom of the lower upsetting die 7 is of the same diameter as the blank 1, permitting the blank to be placed therein and properly centered as shown in Fig. 3. The blank 1 is heated to a red heat and placed in the lower upsetting die as shown in Fig. 3.

When the upper die descends upon the blank shown in Fig. 3, the blank will be upset, assuming the barrel shape or double truncated conical shape as shown at 12 in Figs. 4 and 5, the point 9 in the upper upsetting die forming a centering socket 13 in the upper end of the blank.

As shown in Figs. 4 and 5, the outer refined grain 10 will be caused to flow outward toward the peripheral center of the uncompleted product, the axial, less refined grain remaining through the axial center thereof as shown at 11.

The product 12, while still hot, is then inverted and placed in the lower forging die which is shaped as shown at 14, and provided in its bottom with a centering point 15 which receives the socket 13 of the blank. The lower portion 16 of the lower forging die is of a size to fit the adjacent end of the blank 12, as shown in Fig. 5.

The upper forging die 17 is provided in its top with a centering point 18. As the upper forging die descends, the blank will be forged into the completed gear blank shown at 19, the refined grain 10 of the metal flowing outward from the hub portions 20 to the teeth portion 21, while the less refined grain 11 remains through the axial center of the gear blank.

The centering point 18 will form a socket 22 in the axial center of the gear blank upon the side opposite to the socket 13 providing means for easily centering the blank for machining the same.

As best shown in Fig. 7, all of the refined portion of the grain of the metal flows outward from the hub portions into the teeth portion of the gear blank, the axial center of the same containing all of the coarser grain and the imperfections and defects.

This central portion of the gear blank may be cut out as shown at 23 in the finished gear 24 illustrated in Fig. 8, the teeth 25 being cut from the refined grain 21 of the metal, this grain flowing outward from the hub portions 20 of the gear, forming the strongest possible tooth construction.

I claim:

1. The method of forming gear blanks consisting in cutting a flat ended blank from a bar, said blank having a length greater than the diameter thereof, upsetting the blank endwise producing a barrel shaped product and placing the barrel shaped product in a forging die and forging the same endwise, causing the outer grain of the blank to flow outward from the hub portions into the teeth portion of the gear blank.

2. The method of forming gear blanks consisting in cutting a flat ended blank from a bar, said blank having a length greater than the diameter thereof, upsetting the blank endwise, producing a barrel shaped product, inverting said product in a forging die and forging the same endwise, causing the outer grain of the blank to flow outward from the hub portions into the teeth portion of the gear blank.

3. The method of forming gear blanks consisting in cutting a flat ended blank from a bar, said blank having a length greater than the diameter thereof, heating the blank, upsetting the blank endwise producing a barrel shaped product, placing the product in a forging die while still hot and forging the same endwise, causing the outer grain of the blank to flow outward from the hub portions into the teeth portion of the gear blank.

4. The method of forming gear blanks consisting in cutting a flat ended blank from a bar, said blank having a length greater than the diameter thereof, heating the blank, upsetting the blank endwise, producing a barrel shaped product, placing said product in a forging die while still hot and forging the same endwise, causing the outer grain of the blank to flow from the hub portions into the teeth portion of the gear blank.

CHARLES A. BRAUCHLER.